

# UNITED STATES PATENT OFFICE.

WILLIAM A. McADAMS, OF BAY SHORE, NEW YORK.

## ALUMINUM ALLOY.

1,121,269.

Specification of Letters Patent. Patented Dec. 15, 1914.

No Drawing.

Application filed April 15, 1914. Serial No. 832,052.

*To all whom it may concern:*

Be it known that I, WILLIAM A. McADAMS, a citizen of the United States, and resident of Bay Shore, in the county of Suffolk and State of New York, have invented a new and useful Improvement in Aluminum Alloys, of which the following is a specification.

My invention relates to an aluminum alloy with the object in view of providing a very soft alloy suitable for making metal foil.

With this end in view, my invention consists of an aluminum alloy composed of aluminum, cadmium and tin, in which the amount by weight of cadmium exceeds the amount of tin and the amount by weight of aluminum exceeds the amount of cadmium. These several elements are preferably combined in substantially the following proportions by weight, namely, one hundred parts aluminum, thirty parts cadmium and five parts tin. In practically combining these metals, a portion of the aluminum is melted and raised to a heat sufficient to fuse the cadmium, the cadmium is then introduced and after the mass has been somewhat cooled, the tin is introduced, great care being taken to thoroughly agitate the mass during the introduction of the several ele-

ments. The mass may then be poured into the form of ingots to be shipped to points where it is to be used or to be submitted to the rolling action to reduce it to foil. It is very soft and may be rolled into thin sheets 35 which may be manipulated similar to the manipulations of what is known in the art as tin foil.

What I claim is:

1. An aluminum alloy composed of aluminum, cadmium and tin, in which the proportion of cadmium exceeds by weight the proportion of tin and the proportion of aluminum exceeds by weight the proportion of cadmium. 40 45

2. An aluminum alloy composed of aluminum, cadmium and tin combined in substantially the following proportions by weight, namely, one hundred parts aluminum, thirty parts cadmium and five parts 50 tin. 50

In testimony, that I claim the foregoing as my invention, I have signed my name in presence of two witnesses, this 14th day of April, 1914.

WILLIAM A. McADAMS.

Witnesses:

F. GEORGE BARRY,  
LIDA M. EGBERT.